

Patented Mar. 22, 1938

2,111,893

# UNITED STATES PATENT OFFICE

2,111,893

## METHOD OF MAKING STEEL

Clarence D. King, Brooklyn, N. Y., assignor to  
United States Steel Corporation, New York,  
N. Y., a corporation of New Jersey

No Drawing. Application May 29, 1936,  
Serial No. 82,652

4 Claims. (Cl. 75—46)

This invention relates to an improved steel-making process and more particularly to a method of producing low phosphorus steel from high phosphorus steel. This application is a continuation-in-part of my prior application Serial No. 10,715, filed March 12, 1935.

When pig iron is "blown" or oxidized, as in the Bessemer process, the initial phosphorus in the pig iron of between .07—.10% is raised to between approximately .075—.110% due to the elimination of various metalloids such as carbon, manganese, and silicon. No phosphorus is eliminated from the metal in the process. Steels containing phosphorus contents of this order, .08—.11%, are much stiffer than basic open hearth steels with the same carbon and manganese contents. Bessemer steels by reason of the lack of ductility are, therefore, limited in their useful applications.

It is well known that in the presence of oxidizing and basic slags the phosphorus content of molten steel baths can be lowered. In the presence of calcium oxide, the phosphorus pentoxide obtained by the action of phosphorus with iron oxide forms a relatively stable calcium phosphate compound in accordance with the following reactions:



The usual basic materials employed are limestone or lime, and the usual oxidizing materials employed are ore, roll scale, cinder, etc. These melt down together to form slags. These materials must be converted into liquid form before the phosphorus reaction may be obtained. In basic open hearth and basic electric furnace processes the above materials are incorporated as part of the charge. Special methods of dephosphorizing Bessemer steel have been proposed whereby the aforesaid basic and oxidizing materials mixed in various proportions are added to the ladle and the steel to be dephosphorized is poured thereon or therethrough. These materials, when once used and converted into a molten form (slag), cannot be again used for dephosphorizing subsequent heats.

The use of special mixtures of basic and oxidizing materials for dephosphorizing purposes and the restriction of the mixture to a single use is highly undesirable from an economic standpoint, wherein the initial cost of the materials is a relatively small item. The heating to fusion in separate vessels, the apportioning of definite amounts of the fused material for given masses of molten metal, the practice of the dephosphorizing process on a relatively small scale, are factors which largely increase the costs of such processes.

One of the objects of the present invention is to provide a relatively simple, cheap and effective process for the dephosphorizing of Bessemer or

other high phosphorus steels. Another object is to provide a relatively inexpensive and efficient slag composition effective for the dephosphorizing of steels containing relatively high phosphorus. Another object is to provide a process effective for dephosphorizing high phosphorus steels on a large scale basis. Other objects and advantages will be apparent as the invention is more fully disclosed.

In accordance with these objects I have found that the end slag product of the usual open hearth furnace wherein a low carbon basic steel has been produced is admirably suitable for the dephosphorizing of high phosphorus steels particularly those steels which are in the highly oxidized condition which Bessemer steels are in at the conclusion of the oxidizing blow. I have further found that these slags have a relatively high power of absorbing phosphorus and that consequently they may be repeatedly employed as dephosphorizing agents.

I therefore propose a new method for manufacturing low phosphorus steels which essentially comprises a duplex process wherein I first produce a melt in a regenerative furnace of basic low carbon steel in accordance with standard practice, withdraw the melt, retaining the slag on the hearth, and then charge repeatedly into the furnace a number of melts of oxidized high phosphorus steel, retaining each charge in contact with the slag to permit the dephosphorizing reaction to proceed to completion, and withdrawing each charge at the conclusion of this time interval into a ladle or other suitable vessel for the addition thereto of such other constituents as may be desired in the steel, such as manganese, aluminum, silicon, etc.

The phosphorus absorbing properties of the slag in the furnace gradually become lowered and when the slag is unable to remove the phosphorus from the molten metal down to the point desired, the slag is withdrawn from the furnace and a second melt of low carbon basic steel is made therein. The slag resulting is then utilized to dephosphorize further successive melts or increments of oxidized Bessemer steel in the same manner as heretofore described. Thus the process of the present invention may be practiced as a continuous process of manufacturing low phosphorus steels.

By my process I have been able to lower the phosphorus content of Bessemer blown metal (steel) containing between .075 to .110% phosphorus down to as low as .010% phosphorus, the steel so produced possessing required physical properties for useful employment in products not now satisfactorily served by present types of Bessemer steels.

The slag or end product of a low carbon basic open hearth steel, due to the fact that the car-

bon is oxidized by means of the slag, must necessarily be highly oxidizing. It is also true that such slags are also very basic. Characteristic open hearth slags from low carbon steel are as follows:

|                         | Per cent  |
|-------------------------|-----------|
| Silica                  | 8 -12     |
| Iron oxide              | 25 -40    |
| Manganese               | 5 -10     |
| 10 Phosphorus pentoxide | 1.5 - 2.0 |
| Alumina and titania     | 1.5 - 2.5 |
| Lime                    | 35 -50    |
| Sulphur                 | .1 - .2   |

In order to satisfy the  $SiO_2$  and  $P_2O_5$  contents 15 of the slag itself, a certain amount of the lime ( $CaO$ ) is required. For each part (by weight) of  $SiO_2$  in the slag approximately 1.86 parts  $CaO$  is required. A low carbon slag usually contains  $SiO_2$ -12%;  $CaO$ -43%;  $FeO$  total-30%; 20  $P_2O_5$ -2%. In such a slag there is available an excess  $CaO$  content of 24.70% beyond that required for satisfying the silica ( $SiO_2$ ) and the phosphorus ( $P_2O_5$ ) content of the slag. The slag, therefore, is extremely basic. Slags of this character are also highly oxidizing as indicated by 25 the iron oxide content of the slag and, therefore, useful in dephosphorizing Bessemer or other steels.

In accordance with the present invention the 30 method is practiced preferably as follows:

A tilting basic open hearth furnace is preferably used in the practice of the present invention. A standard basic low carbon steel is made therein by standard practices. Such standard 35 practice may be varied widely as one skilled in the art will recognize. The furnace is charged with pig iron (hot metal), "blown" metal together with lime, limestone and ore each in proportions suitable for the purpose and the charge 40 is melted down. As an example, three typical charges are listed below:

| 45                     |  | Percent of materials used per ton metallic charge |           |            |       |
|------------------------|--|---------------------------------------------------|-----------|------------|-------|
|                        |  | Charge I                                          | Charge II | Charge III |       |
| Fe in ore, scale, etc. |  | 1.5                                               | 4.5       |            | 80.0  |
| Blown metal            |  | 85.0                                              | 61.8      |            | 12.0  |
| Hot metal              |  |                                                   |           |            | 3.3   |
| Cold iron              |  | 63.0                                              | 33.3      |            | 4.0   |
| Steel scrap            |  | 0.5                                               | 0.4       |            | 0.7   |
| Additions              |  |                                                   |           |            |       |
| Total metallic charge  |  | 100.0                                             | 100.0     |            | 100.0 |
| Limestone              |  | 5.00                                              | 6.00      |            | 5.55  |
| Dolomite               |  | 2.50                                              | 2.37      |            | 1.53  |
| Fluorspar              |  | .20                                               | .28       |            | .15   |

The resultant slags are highly oxidizing and basic and have the composition above indicated.

The molten low carbon steel thus formed is 60 tapped out of the tilting furnace in customary manner but the molten or end slag is retained in the furnace. To the furnace is then added a charge of "blown" or oxidized high phosphorus steel such as blown Bessemer steel. A reaction 65 immediately takes place between the blown metal and the slag and dephosphorization of the steel is effected thereby. If required, a small amount of "hot metal" or pig iron is added to accelerate and increase the reaction. The rapidity of the 70 process depends largely upon the rapidity of getting the blown metal into the furnace, since the process itself is to all intents and purposes instantaneous.

The charge having now been dephosphorized, is 75 tapped out of the furnace, but the slag is still

retained in the furnace, only enough of this slag being voided from the furnace to cover the steel ladle in the customary manner. The furnace is again charged with more "blown" metal and the process repeated again and again until the slag becomes ineffective to reduce the phosphorus content of the blown metal to the extent desired. The slag then is removed and a second melt of basic open hearth steel is made in the furnace and the end slag thereof is retained therein 10 when the melt is tapped out.

Each successive charge of dephosphorized metal after tapping from the furnace may be treated in the ladle with various addition materials and alloying constituents, such as manganese, silicon, carbon, aluminum, etc. to form 15 the steel composition desired.

If any siliceous Bessemer slag is accidentally charged into the tilting furnace along with the "blown" metal, only sufficient lime is introduced 20 into the bath to compensate for this extra silica ( $SiO_2$ ). By this process it is possible to use an extremely small amount of slag to effect the required dephosphorization of a relatively large 25 volume of oxidized high phosphorus steel through repeated use of the initial end slag of the basic open hearth furnace.

The following example illustrates the repetitive character of the process. After a low carbon 30 heat was made on a 150-ton basic open hearth tilting furnace, the final slag of that heat which was retained in the furnace, weighed 24,000 pounds and analyzed as follows:

|                                | Per cent |
|--------------------------------|----------|
| CaO                            | 48 35    |
| SiO <sub>2</sub>               | 12       |
| P <sub>2</sub> O <sub>5</sub>  | 2        |
| FeO                            | 11.7     |
| Fe <sub>2</sub> O <sub>3</sub> | 11.3     |
| MgO                            | 7 40     |

To this slag I added four successive batches or melts of "blown" Bessemer steel as follows:

| Heat #1                 |                            |                         |     |      |      |      |
|-------------------------|----------------------------|-------------------------|-----|------|------|------|
| Time charged in furnace | Weight of blown metal      | Analysis of blown metal |     |      |      |      |
|                         |                            | O                       | Mn  | P    | S    | Si   |
| 12:19 p. m.             | 117, 100                   | .05                     | .03 | .080 | .028 | .003 |
| 12:43 p. m.             | 117, 000                   | .05                     | .03 | .076 | .027 | .003 |
| 1: 05 p. m.             | 116, 600                   | .03                     | .04 | .074 | .028 | .003 |
| 1: 39 p. m.             | 6,000 Hot metal (pig iron) | 3.75                    | .61 | .080 | .028 | 1.79 |

  

| Final steel analysis                       |     |     |      |      |       |
|--------------------------------------------|-----|-----|------|------|-------|
| Tapped 1:36 p. m. and ladle additions made | .05 | .29 | .014 | .025 | ----- |

| Heat #2                 |                            |                         |     |      |      |      |
|-------------------------|----------------------------|-------------------------|-----|------|------|------|
| Time charged in furnace | Weight of blown metal      | Analysis of blown metal |     |      |      |      |
|                         |                            | O                       | Mn  | P    | S    | Si   |
| 2:01 p. m.              | 124,800                    | .03                     | .04 | .076 | .027 | .002 |
| 2:26 p. m.              | 112,800                    | .03                     | .03 | .076 | .029 | .002 |
| 2:47 p. m.              | 112,000                    | .03                     | .03 | .076 | .030 | .004 |
| 3:00 p. m.              | 4,000 hot metal (pig iron) | 3.83                    | .63 | .078 | .029 | 1.65 |

  

| Final steel analysis                       |     |     |      |      |       |
|--------------------------------------------|-----|-----|------|------|-------|
| Tapped 3:16 p. m. and ladle additions made | .05 | .30 | .024 | .025 | ----- |

## Heat #3

| 5                                             | Time charged in furnace | Weight of blown metal       | Analysis of blown metal |      |       |       |      |
|-----------------------------------------------|-------------------------|-----------------------------|-------------------------|------|-------|-------|------|
|                                               |                         |                             | C                       | Mn   | P     | S     | Si   |
| 3:44 p. m.                                    |                         | 124,900                     | .03                     | .04  | .079  | .034  | .002 |
| 3:57 p. m.                                    |                         | 5,000 hot metal (pig iron). | 3.94                    | .61  | .081  | .033  | 1.50 |
| 10 4:07 p. m.                                 |                         | 124,800                     | .04                     | .05  | .073  | .030  | 1.50 |
|                                               |                         |                             | Final steel analysis    |      |       |       |      |
| 15 Tapped 4:24 p. m. and ladle additions made |                         |                             | 0.05                    | 0.29 | 0.025 | 0.030 |      |

## Heat #4

| 20                   | Time charged in furnace | Weight of blown metal       | Analysis of blown metal |     |      |      |      |
|----------------------|-------------------------|-----------------------------|-------------------------|-----|------|------|------|
|                      |                         |                             | C                       | Mn  | P    | S    | Si   |
| 25 5:57 p. m.        |                         | 125,000                     | .03                     | .03 | .078 | .034 | .004 |
| 6:13 p. m.           |                         | 5,200 hot metal (pig iron). | 3.93                    | .62 | .073 | .030 | 1.50 |
| 6:23 p. m.           |                         | 124,700                     | .04                     | .04 | .074 | .037 | .005 |
|                      |                         |                             | Final steel analysis    |     |      |      |      |
| 30 Tapped 6:37 p. m. |                         |                             | .06                     | .32 | .025 | .027 |      |

|    |                                                    | Pounds    |
|----|----------------------------------------------------|-----------|
| 35 | Total metal charged in furnace                     | 1,220,800 |
|    | Total ferro-alloys added to steel ladles           | 11,500    |
|    | Gross total metal used                             | 1,232,300 |
|    | Weight of ingots produced                          | 1,196,000 |
| 40 | Weight of scrap produced (skulls, pit scrap, etc.) | 17,100    |
|    |                                                    | Per cent  |
| 45 | Yield from charge to ingots                        | 97.05     |
|    | Scrap produced                                     | 1.39      |
|    | Loss                                               | 1.56      |

| 50         | Total weight of ingots (gross tons) | Time of heat  | Tons ingots per hour melting time |
|------------|-------------------------------------|---------------|-----------------------------------|
| Heat No. 1 | 148                                 | 1 hr. 17 min. | 115.4                             |
| Heat No. 2 | 156                                 | 1 hr. 15 min. | 124.8                             |
| Heat No. 3 | 114                                 | 0 hr. 40 min. | 170.9                             |
| Heat No. 4 | 116                                 | 0 hr. 40 min. | 173.9                             |

|                                                             |                 |
|-------------------------------------------------------------|-----------------|
| Total production                                            | 534 tons        |
| Total over-all time required including delays between heats | 6 hrs. 18 mins. |
| 60 Grand total production per operating hour                | 84.8 tons       |

The temperature of the "blown" or oxidized high phosphorus metal as it comes from the converter is relatively high and when charged directly into the open hearth furnace no additional heat energy other than that required to keep the slag molten and the furnace up to operating temperature need be added. As a result, the fuel consumption in my process is extremely low. The process can be operated with 500,000 B. t. u. or less per ton of ingots produced. A comparison of the fuel consumption with the 75 process described in this application as against

standard methods shows a striking economy in fuel consumption:

|                                          | Standard basic open hearth practice | Standard duplex practice | Practice as herein described | 5 |
|------------------------------------------|-------------------------------------|--------------------------|------------------------------|---|
| Normal gross B. t. u. per ton of ingots. | 4,000,000 to 5,000,000              | 2,000,000 to 3,000,000   | 400,000 to 700,000           |   |

A further decided advantage of the process is the greatly increased production possible from basic open hearth furnaces. Since the process is extremely rapid, as much as 100 tons or more of dephosphorized steel can be obtained per hour. The following indicates the normal productive capacity of 150-ton furnaces with various processes:

*Comparison of ingot production per hour on 150-ton furnaces with various processes*

| Standard basic open hearth | Standard duplex | Practice as described herein | 20 |
|----------------------------|-----------------|------------------------------|----|
| 14 to 17 tons              | 20 to 40 tons   | 85 to 125 tons.              | 25 |

From the above description it is apparent that the present invention affords an extremely economical and rapid method of manufacturing low phosphorus steels from high phosphorus metal.

Having broadly described the present invention and given one specific embodiment thereof, it is apparent that there may be modifications and adaptations made therein without departing from the nature and scope thereof and all such modifications and adaptations are contemplated as may fall within the scope of the following claims.

What I claim is:

1. The method of manufacturing low phosphorus steel which comprises producing in a basic open hearth furnace a melt of basic low carbon steel in accordance with standard practice utilizing the usual basic and oxidizing slag therein, removing this melt, leaving the molten slag in the furnace, adding to the furnace blown Bessemer metal, holding the same in contact with the molten slag for a sufficient time interval to obtain the removal of phosphorus from the metal, tapping the metal from the furnace, adding a second batch of blown Bessemer metal to the furnace and treating it similarly to the first batch, tapping the same, and making further additions of metal to the furnace until the slag in the furnace becomes saturated with phosphorus to the extent that the treated Bessemer metal retains an undesirable amount of phosphorus, tapping then the said slag and producing a second melt of basic low carbon steel as before and treating further batches of blown Bessemer steel with the second slag to dephosphorize the same until the second slag is similarly saturated with phosphorus, continuing the said process ad infinitum, the treated dephosphorized Bessemer steel resulting being adjusted by suitable ferro-alloy additions to a desired composition prior to casting.

2. A dephosphorizing slag composition for use in the removal of phosphorus from blown Bessemer steel comprising a basic and oxidizing slag characteristic of and resulting as an end product in the manufacture of low carbon steel by standard practices in a basic open hearth furnace, said slag containing between 8% and 12% silica, 35% and 50% lime, 25% and 40% iron oxide, 5% and 10% manganese oxide, 1.5% and 2.0% phosphorus pentoxide, 1.5% and 2.5% of aluminum and tita-

nium oxides combined, and .10% and .20% sulphur.

3. The method of manufacturing low phosphorus steel from blown Bessemer metal which comprises forming a melt of basic low carbon steel in a regenerative furnace, removing the melt retaining the end slag product in the furnace, charging the blown Bessemer metal into the said furnace onto said retained slag and withdrawing the charge from the furnace after a time interval adapted to permit the said slag to remove phosphorus and other oxidized impurities from the said blown metal.

4. The method of manufacturing low phosphorus steel from blown Bessemer metal which comprises forming a melt of basic low carbon steel in a regenerative furnace, removing the melt retaining the end slag product in the furnace, 5 and charging a succession of batches of said blown Bessemer metal into said furnace onto said retained slag and withdrawing each charge from the furnace after a time interval adapted to permit the slag to remove the phosphorus and other 10 oxidized impurities from the said blown metal.

CLARENCE D. KING.